

May 1, 1962

K. SIXTUS ET AL  
COMPOSITION OF MAGNETIC CORE MATERIAL  
AND METHOD OF PRODUCING SAME  
Filed June 4, 1959

3,032,503



Inventors:

KLAUS SIXTUS  
KARL REICHEL

By *Toulmin & Toulmin*

Attorneys

3,032,503

COMPOSITION OF MAGNETIC CORE MATERIAL  
AND METHOD OF PRODUCING SAMEKlaus Sixtus, Bad Homburg, and Karl Reichel, Kelkheim  
(Taunus), Germany, assignors to Licentia Patent-Ver-  
waltungs-G.m.b.H., Hamburg, Germany

Filed June 4, 1959, Ser. No. 818,126

Claims priority, application Germany June 4, 1958  
6 Claims. (Cl. 252—62.5)

The present invention relates to a new composition of magnetic core material and method of producing the same. More in particular, the present invention relates to a new composition of magnetic core material and a method of producing such magnetic core material having a substantially rectangular hysteresis loop.

Magnetic core material having a substantially rectangular hysteresis loop is used for example, in switches, for storage purposes, or in magnetic amplifiers.

It has already become known to provide core material having a substantially rectangular hysteresis loop comprising magnetizable ceramic material containing iron oxide, magnesium oxide, and manganese oxide.

The particular composition of these known core materials and the method of producing such magnetic core materials has proved, however, unsatisfactory, complicated and costly.

These known core materials have a hysteresis loop which is characterized by a peak induction  $B_s$  of from 1500 to 2000 gauss, a coercive force of from 0.7 to 2 oersteds, and a remanence-peak induction ratio  $B_r:B_s=0.85$  to 0.95, and a squareness ratio  $R_s=0.8$  to 0.9.  $R_s$  is defined by the equation

$$R_s = \frac{B_1 \left( \text{at } -\frac{H_m}{2} \right)}{B_s \left( \text{at } H_m \right)}$$

$B_s$  being the induction obtained by maximum modulation of the loop up to field intensity  $H_m$ ,  $B_1$  being the induction at a field intensity of

$$-\frac{H_m}{2}$$

According to another improved method of producing core material, ferrites on an iron oxide and cobalt oxide basis are subjected to the influence of heat and a magnetic field. However, this method and the core material so obtained still are unsatisfactory. According to this known method a hysteresis loop is obtained having a remanence  $B_r$  of up to 3000 gauss, a coercive force of from 5 to 80 oersteds, and a squareness ratio  $R_s$  from 0.5 to 0.95. Even these values are obtained only in the direction in which the core material has been exposed to the magnetic field during heat treatment, whereas the hysteresis loop has retained its normal, S-shaped configuration in all other directions.

All these known core materials and the methods of producing them are unsatisfactory. In addition to a rectangular hysteresis loop it is extremely desirable for several purposes to have a high remanence but at the same time a low coercive force. Such core materials are used, for example, in magnetic amplifiers, in switching and counting devices and in digital computers. The known core materials, their particular composition and the methods for producing them do not meet these requirements. They do not accomplish the triple purpose of providing for core materials having, at the same time, a substantially rectangular hysteresis loop, a high remanence and a low coercive force. Moreover, the last mentioned method of exposing the core material to the influence of heat and a magnetic field is complicated and costly.

With the foregoing in mind, it is an object of the present invention to provide for a new composition of magnetic core material, which has a substantially rectangular hysteresis loop and, at the same time, both a high remanence and a low coercive force.

It is another object of the invention to provide for a simple and effective method of producing magnetic core material having a substantially rectangular hysteresis loop, a high remanence, and a low coercive force.

These objects are achieved by the present invention, which has found a new composition of core material to be highly superior to any of the known compositions. According to the invention, the core material is composed of the following materials in the following ratio:

0.8 to 1 mol  $Fe_2O_3$ :0.4 to 0.7 mol  $ZnO$ :0.001 to 0.05 mol  $CoO$ , plus a predetermined amount of  $NiO$  so that the mol total of  $ZnO$ ,  $CoO$ , and  $NiO$  is one.

According to another, preferred embodiment of the composition of core material of the present invention, the material contains, in addition to aforescribed substances and amounts,  $CuO$  in an amount of up to 20 mol-percent of the total; in this case the mol total of  $ZnO$ ,  $CoO$ ,  $NiO$  and  $CuO$  is one. The mol ratio between the iron oxide and the total of the other oxides is in the range of from 0.8 to 1:1.

The presence of copper oxide ( $CuO$ ) greatly facilitates the sintering process, referred to further below, without substantially impairing the excellent magnetic characteristics of the core material.

It has been discovered that ferrites with a smaller percentage of iron oxide ( $Fe_2O_3$ ) than the stoichiometric composition will produce a substantially rectangular hysteresis loop, without requiring a treatment in a magnetic field and exposure to heat. This is particularly true where the abovementioned composition of the invention is chosen. The new method for producing a magnetic core material with a substantially rectangular hysteresis loop, a high remanence and a low coercive force can therefore dispense with this step of exposing the material to heat in a magnetic field. According to the method of the present invention, the metal oxides or compounds giving off the oxides when heated, are pulverized, mixed and subjected to a first sintering process in air and at a temperature of from 800 to 1000° C.,

whereupon the cores are molded, which are then subjected to a second, main sintering operation in oxygen and at a temperature of from 1200 to 1400° C.

According to another embodiment of the method of the invention, the cobalt compound, which is to furnish the necessary share of  $CoO$  in the core material is added only after the other substances have gone through the abovementioned first sintering operation.

More in detail, a certain quantity of iron oxide is mixed, for example with nickel carbonate, zinc carbonate and cobalt carbonate of such quantities, that the aforescribed mol ratio is obtained. The mixture is then finely ground, with water being added, in a grinding mill as, e.g., a ball mill. Two hours will be sufficient to effect this wet grinding operation. This finely ground mixture is then dried. Thereafter, it is exposed to a first sintering process. The sintering is done in air or oxygen at a temperature taken from the range of from 800 to 1000° C., and for a period of about two hours. The sintered product is ground again in a suitable grinding mill, such as a ball mill, with water being added. The product is dried and then used as the material for molding annular cores, in a manner known per se. These cores are then subjected to a second, main sintering operation, which is done in oxygen and at a temperature of from 1200 to 1400° C.

The invention will be even better appreciated upon

reading the following examples in conjunction with the accompanying drawing, which is a diagram showing the advantageous characteristics of the core material of the composition and produced according to the method of the present invention.

*Example I*

58.3 grams iron oxide ( $Fe_2O_3$ ), 17.85 grams nickel carbonate, 24.4 grams zinc carbonate and 2.1 grams cobalt carbonate are taken, which amounts correspond to the mol ratio of 0.98 mol  $Fe_2O_3$ :0.37 mol NiO:0.58 mol ZnO:0.05 mol CoO. These substances are mixed in a ball mill for about two hours during which process water is added. The mixture is then removed from the ball mill and dried. Thereafter, the dried mixture is sintered for a first time for two hours at 950° C. in air. The sintered product is then wet ground in a ball mill and thereafter dried again. Thereupon the dried product is subjected to a pressure of 0.5 ton/cm.<sup>2</sup> in a mold and shaped into an annular core. The core is then subjected to a second, final, sintering process for about two hours at a temperature of 1250° C., this time not exposed to air but to oxygen. Thereafter it is cooled in the sintering oven proper.

The characteristics of the hysteresis loop of the annular core obtained by this treatment are shown in the accompanying drawing and are as follows:  $B_s$ =3100 gauss; coercive force  $H_c$ =0.75 oersted; ratio  $B_r/B_s$ =0.97; squareness ratio  $R_s$ =0.94. The specific electric resistance is  $10^9\Omega$  centimeters.

*Example II*

553 grams iron oxide ( $Fe_2O_3$ ), 183.2 grams nickel carbonate and 243.8 grams zinc carbonate are mixed with water for about two hours, whereupon the mixture is dried. The dried mixture is then exposed to a first sintering process in oxygen at a temperature of 900° C. and for a period of two hours. To 100 grams of this mixture there are added 2.1 grams cobalt carbonate and 1.7 grams iron oxide ( $Fe_2O_3$ ) so as to obtain a composition having a ratio of 0.96 mol  $Fe_2O_3$ :0.38 mol NiO:0.58 mol ZnO:0.04 mol CoO. The mixture is then wet ground and dried. The ground and dried product is then pressed as in Example I to the shape of an annular core. The annular cores are then sintered in oxygen at a temperature of 1250° C. for two hours.

A magnetic core material is obtained having a substantially rectangular hysteresis loop with the following characteristics:  $B_s$ =2540 gauss;  $H_c$ =0.85 oersted, ratio  $B_r/B_s$ =0.96;  $R_s$ =0.93. The specific electric resistance is  $2.10^{11}\Omega$  centimeters.

*Example III*

553 grams iron oxide ( $Fe_2O_3$ ), 183.2 grams nickel carbonate and 243.8 grams zinc carbonate are mixed, dried and sintered in oxygen for two hours at a temperature of 900° C. To 100 grams of this sintered mixture there are added 0.64 gram cobalt carbonate and 2.2 grams iron oxide so as to have a composition with the ratio of 0.98 mol  $Fe_2O_3$ :0.398 mol NiO:0.59 mol ZnO:0.012 mol CoO. This mixture is then wet ground and dried whereupon the annular cores are formed. These are then exposed to a sintering process in oxygen at a temperature of 1250° C. and for a period of two hours.

The hysteresis loop of the magnetic core has the following characteristics:  $B_s$ =2900 gauss;  $H_c$ =0.5 oersted; ratio  $B_r/B_s$ =0.95;  $R_s$ =0.83.

The foregoing examples, in conjunction with the accompanying diagram show, that magnetic cores are obtained having an excellently rectangular hysteresis loop with high remanence and, at the same time, a low coercive force. This is obtained even though the cores were not subjected to heat in a magnetic field.

It will be understood that this invention is susceptible

to further modification and, accordingly, it is desired to comprehend such modifications within this invention as may fall within the scope of the appended claims.

What we claim is:

- 5 1. As a composition of matter, magnetic core material having a substantially rectangular hysteresis loop, composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO, and NiO is one.
- 10 2. As a composition of matter, magnetic core material as described in claim 1, further containing copper oxide in an amount of up to 20 mol-percent of the entire composition, the mol total of ZnO, CoO, NiO and CuO being one.
- 15 3. A method for producing magnetic core material having a substantially rectangular hysteresis loop and being composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO, and NiO is one, comprising the steps of pulverizing and mixing  $Fe_2O_3$ , ZnO, CoO and NiO, subjecting the same to a first sintering process in air at a temperature of from 800 to 1000° C., molding the magnetic cores, and subjecting the latter to a second, main sintering process in oxygen at a temperature of from 1200 to 1400° C.
- 20 4. A method for producing magnetic core material having a substantially rectangular hysteresis loop and being composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO and NiO is one, comprising the steps of pulverizing and mixing  $Fe_2O_3$ , ZnO and NiO, subjecting the same to a first sintering process in air at a temperature of from 800 to 1000° C., adding a predetermined amount of cobalt carbonate to the sintered product, molding the magnetic cores, and subjecting the latter to a second, main sintering process in oxygen at a temperature of from 1200 to 1400° C.
- 25 5. A method for producing magnetic core material having a substantially rectangular hysteresis loop and being composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO and NiO is one, comprising the steps of pulverizing and mixing iron oxide ( $Fe_2O_3$ ), nickel carbonate, zinc carbonate and cobalt carbonate, subjecting the same to a first sintering process in air at a temperature of from 800° to 1000° C., molding the magnetic cores, and subjecting the latter to a second main sintering process in oxygen at a temperature of from 1200° to 1400° C.
- 30 6. A method for producing magnetic core material having a substantially rectangular hysteresis loop and being composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO and NiO is one, comprising the steps of pulverizing and mixing iron oxide ( $Fe_2O_3$ ), nickel carbonate and zinc carbonate, subjecting the same to a first sintering process in air at a temperature of from 800° to 1000° C., adding a predetermined amount of cobalt carbonate to the sintered product, molding the magnetic cores, and subjecting the latter to a second, main sintering process in oxygen at a temperature of from 1200° to 1400° C.
- 35 7. A method for producing magnetic core material having a substantially rectangular hysteresis loop and being composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO and NiO is one, comprising the steps of pulverizing and mixing iron oxide ( $Fe_2O_3$ ), nickel carbonate, zinc carbonate and cobalt carbonate, subjecting the same to a first sintering process in air at a temperature of from 800° to 1000° C., adding a predetermined amount of cobalt carbonate to the sintered product, molding the magnetic cores, and subjecting the latter to a second, main sintering process in oxygen at a temperature of from 1200° to 1400° C.
- 40 8. A method for producing magnetic core material having a substantially rectangular hysteresis loop and being composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO and NiO is one, comprising the steps of pulverizing and mixing iron oxide ( $Fe_2O_3$ ), nickel carbonate, zinc carbonate and cobalt carbonate, subjecting the same to a first sintering process in air at a temperature of from 800° to 1000° C., adding a predetermined amount of cobalt carbonate to the sintered product, molding the magnetic cores, and subjecting the latter to a second, main sintering process in oxygen at a temperature of from 1200° to 1400° C.
- 45 9. A method for producing magnetic core material having a substantially rectangular hysteresis loop and being composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO and NiO is one, comprising the steps of pulverizing and mixing iron oxide ( $Fe_2O_3$ ), nickel carbonate, zinc carbonate and cobalt carbonate, subjecting the same to a first sintering process in air at a temperature of from 800° to 1000° C., adding a predetermined amount of cobalt carbonate to the sintered product, molding the magnetic cores, and subjecting the latter to a second, main sintering process in oxygen at a temperature of from 1200° to 1400° C.
- 50 10. A method for producing magnetic core material having a substantially rectangular hysteresis loop and being composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO and NiO is one, comprising the steps of pulverizing and mixing iron oxide ( $Fe_2O_3$ ), nickel carbonate, zinc carbonate and cobalt carbonate, subjecting the same to a first sintering process in air at a temperature of from 800° to 1000° C., adding a predetermined amount of cobalt carbonate to the sintered product, molding the magnetic cores, and subjecting the latter to a second, main sintering process in oxygen at a temperature of from 1200° to 1400° C.
- 55 11. A method for producing magnetic core material having a substantially rectangular hysteresis loop and being composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO and NiO is one, comprising the steps of pulverizing and mixing iron oxide ( $Fe_2O_3$ ), nickel carbonate, zinc carbonate and cobalt carbonate, subjecting the same to a first sintering process in air at a temperature of from 800° to 1000° C., adding a predetermined amount of cobalt carbonate to the sintered product, molding the magnetic cores, and subjecting the latter to a second, main sintering process in oxygen at a temperature of from 1200° to 1400° C.
- 60 12. A method for producing magnetic core material having a substantially rectangular hysteresis loop and being composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO and NiO is one, comprising the steps of pulverizing and mixing iron oxide ( $Fe_2O_3$ ), nickel carbonate, zinc carbonate and cobalt carbonate, subjecting the same to a first sintering process in air at a temperature of from 800° to 1000° C., adding a predetermined amount of cobalt carbonate to the sintered product, molding the magnetic cores, and subjecting the latter to a second, main sintering process in oxygen at a temperature of from 1200° to 1400° C.
- 65 13. A method for producing magnetic core material having a substantially rectangular hysteresis loop and being composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO and NiO is one, comprising the steps of pulverizing and mixing iron oxide ( $Fe_2O_3$ ), nickel carbonate, zinc carbonate and cobalt carbonate, subjecting the same to a first sintering process in air at a temperature of from 800° to 1000° C., adding a predetermined amount of cobalt carbonate to the sintered product, molding the magnetic cores, and subjecting the latter to a second, main sintering process in oxygen at a temperature of from 1200° to 1400° C.
- 70 14. A method for producing magnetic core material having a substantially rectangular hysteresis loop and being composed of iron oxide, zinc oxide, cobalt oxide, and nickel oxide in a ratio of from 0.8 to 1 mol  $Fe_2O_3$ :from 0.4 to 0.7 mol ZnO:from 0.001 to 0.05 mol CoO and a determined amount of nickel oxide so that the mol total of the shares of ZnO, CoO and NiO is one, comprising the steps of pulverizing and mixing iron oxide ( $Fe_2O_3$ ), nickel carbonate, zinc carbonate and cobalt carbonate, subjecting the same to a first sintering process in air at a temperature of from 800° to 1000° C., adding a predetermined amount of cobalt carbonate to the sintered product, molding the magnetic cores, and subjecting the latter to a second, main sintering process in oxygen at a temperature of from 1200° to 1400° C.

## References Cited in the file of this patent

UNITED STATES PATENTS

|           |                |               |
|-----------|----------------|---------------|
| 2,656,319 | Berge          | Oct. 20, 1953 |
| 2,723,239 | Harvey         | Nov. 8, 1955  |
| 2,736,708 | Crowley et al. | Feb. 28, 1956 |
| 2,860,105 | Gorter et al.  | Nov. 11, 1958 |

## FOREIGN PATENTS

|               |               |
|---------------|---------------|
| Great Britain | July 11, 1956 |
| France        | Apr. 13, 1955 |
| France        | Feb. 24, 1958 |

## OTHER REFERENCES

RCA Review, Harvey et al., September 1950, pp. 344-347.